

## UNITED STATES PATENT OFFICE

GEORG HANEKOP, OF HANOVER, GERMANY

## GRINDING GRAPHITE

No Drawing. Application filed March 31, 1928, Serial No. 266,444, and in Germany March 16, 1925.

This invention refers broadly to a method of grinding graphite, and in particular the purer grades thereof to a flour-like condition and to thereby obtain a purer and more 5 voluminous and more finely disintegrated powder than generally obtainable heretofore. It has been ascertained by tests made with different grades of commercial graphites that the poorer grades are almost as a rule more 10 finely ground than the superior grades of graphite. This is probably due to the fact that the grinding stones, rollers or equivalent grinding means become better adapted to take hold of the smooth lamellæ or leaves of 15 graphite in the presence of rocks, clay and quartz.

In order to be able to also grind the high-grade kinds of graphite to a flour-like powder I have ascertained by my experiments 20 that such kinds of graphite should be ground with brittle, sand-like substances, but it should be understood that only such kinds of material are suitable for the purpose, as will admit of being removed after the fine 25 grinding, and of these water-soluble salts have been found to be very suitable. Thus ordinary salt or rock-salt have produced very satisfactory results. In case it should be desired to also remove substances from the 30 graphite which are only soluble in acids, salt solutions and the like, such substances may also be added which are not entirely soluble in water, but only in acids, such as low grade potash salts, residues from the extraction of 35 potash and soda-salts and the like. The grinding up of the graphite with the salts may be effected in the dry condition, as well as in the presence of a small amount of water. It should however be noted that only so much 40 water may be added, as will still leave large quantities of the salts undissolved. After the desired degree of fineness has been obtained, the salts are removed by water or by the addition of acids and lixiviation.

45 By treating according to this method for instance the species of graphites known in the trade by the name of "powder-graphite", it has been found that, when treated according to this method, a considerably finer distribution of the particles of graphite may

still be obtained. The graphite thus produced has been found to be particularly adapted for the manufacture of so-called dry cell elements, pocket-lamp-batteries and of similar instrumentalities. If pyrolusite, and particularly artificial pyrolusite, is mixed on the one hand with ordinary commercial powder graphite, and on the other hand with the same kind of graphite which has previously undergone an additional disintegration with 55 the addition of salts, equal amounts of graphite thus treated show an increase of conductivity up to approximately one hundred percent, that is to say almost double the conductivity of the original graphite which has not 60 been ground up with salts.

By the grinding up with salts the graphites become considerably more voluminous, so that larger quantities of pyrolusite or of particles of artificial pyrolusite than heretofore 70 may be enveloped by such treated graphites, as compared with graphites of less fine subdivision.

It should be understood that the scope of the invention is not restricted to the specific 75 details herein recited, but modifications are possible without deviating from the spirit of the invention as defined in the appended claims, and that the highly disintegrated graphite which is the product of this invention 80 is applicable to all the various uses in the arts to which graphite is usually applied.

I claim:—

1. The process of highly disintegrating graphite, which comprises grinding up and 85 treating graphite with salts possessing substantially the physical and chemical properties of rock-salts.

2. The process of highly disintegrating graphite, which comprises intimately grinding 90 graphite with mineral salts possessing substantially the physical and chemical character of ordinary salt and of rock-salt.

3. The process of disintegrating graphite, 95 which consists in intimately grinding graphite with mineral salts of the physical and chemical character of ordinary salt and of rock-salt and in the presence of an insufficiency of solvent, and then removing said salt by treatment with a solvent. 100

4. The process of disintegrating graphite, which consists in grinding graphite and intimately treating it with ordinary neutral salt and thoroughly agitating it therewith, and after a sufficient degree of fineness has been obtained, dissolving the salt and removing it from the graphite.

5. The process of highly disintegrating graphite, which comprises most intimately 10 grinding the graphite with sand-like fragments of mineral salts of the class of ordinary salt and of rock-salt and with an insufficiency of solvent, and after the desired fineness is obtained lixiviating the product and 15 removing the salt.

6. As a new product most highly disintegrated, fluffy, uncolloidal graphite occupying a relatively very large volume as compared with its weight, and suitable for use 20 for batteries and the like.

GEORG HANEKOP.

25

30

35

40

45

50

55

60